

# UNITED STATES PATENT OFFICE.

ROBERT ABBOTT HADFIELD, OF WESTMINSTER, ENGLAND.

## MANUFACTURE OF ALLOY STEEL.

1,362,788.

Specification of Letters Patent. Patented Dec. 21, 1920.

No Drawing.

Application filed May 24, 1920. Serial No. 383,914.

To all whom it may concern:

Be it known that I, Sir ROBERT ABBOTT HADFIELD, Baronet, F. R. S., a subject of the King of Great Britain and Ireland, residing at the city of Westminster, England, have invented Improvements in or Relating to the Manufacture of Alloy Steel, of which the following is a specification.

An advantage of using nickel or chromium, or nickel and chromium, in the manufacture of alloy steels is that the steel is rendered more sensitive to hardening, which, when followed by tempering, enables thicker masses of such steel to be hardened and tempered in a better manner than carbon steel can be hardened and tempered. For example, if a heated mass of carbon steel, say three inches in thickness, be quenched in a cooling medium and then tempered, the first hardening produced by quenching does not penetrate very deeply, consequently the grain of the steel obtained is not properly changed and the subsequent tempering of the steel produces little or no improvement in this respect. When nickel or chromium, or nickel and chromium, is or are used in the manufacture of steel, the hardening penetrates much more deeply, consequently when such hardened steel is afterward tempered, the material is much stiffer in quality.

Now I have discovered as the result of experiments, that the presence of manganese between predetermined percentage limits, in an otherwise carbon steel has a similar influence to nickel or chromium, or both, and that manganese can, under suitable conditions, be used in lieu of these much more expensive metals, to produce an alloy steel capable of being hardened and tempered in an advantageous manner to produce material possessing valuable technical characteristics, among which may be mentioned its power of offering considerable resistance to tensile and shock stresses, such as is offered by nickel steel, chromium steel, and nickel-chromium steel, and which can therefore be used in lieu of these expensive steels for various practical purposes, as for instance in the construction of aeroplanes, motor cars, for instance crank shafts, and so forth where the material is liable to be subjected to considerable tensile and shock stresses.

I have found that a manganese alloy steel, such as referred to, possessing valuable characteristics such as those mentioned, can be obtained when made with from about one

decimal four to three and a half per cent. of manganese and with carbon and silicon comparatively low, and when subjected to a suitable heat treatment. Thus, good results have been obtained with alloy steels containing from about .2% to .3% of carbon, from about .2% to .3% of silicon and from about 1.4 to 2% of manganese, the material being heat treated by heating it to a relatively high temperature, then rapidly cooling it, then reheating it to a lower temperature and then again rapidly cooling it.

According to one example, satisfactory results have been obtained with alloy steels containing in addition to iron, from about .23 to .29% say .3% of carbon, from about .22 to .27% say .3% of silicon and about 1.39% say 1.4% of manganese, sulfur and phosphorus being low, such steels being heat treated by heating them to a temperature of the order of about 800 to 900° C., advantageously about 850° C., then rapidly cooling them, as by quenching them in water, or oil, then reheating them to a temperature of the order of from about 600° C. to 700° C., advantageously about 650° C., and then again quenching them, as in water or oil.

The steel may in some cases be reheated, preparatory to the second quenching, to a temperature of from about 450° C. up to say, about 700° C., instead of from about 600° to 700° C., according to the physical qualities desired and the percentages of carbon and manganese present, and quenched in oil or water, or allowed to cool in the air. If the quenching of the alloy steel is effected in water, the temperature of the steel preparatory to the first quenching may be 20° to 40° lower than when quenching in oil.

In the case for example of small bars of alloy steel of about one and one eighth inches thickness and containing from about 1.4% up to about 2% manganese, satisfactory results have been attained by introducing the bars into a furnace at a temperature of about 850° C. and allowing them to soak at this temperature for about half an hour, then removing them from the furnace and quenching them in water until cold, then reheating them in the furnace at the required lower temperature, say of about 450° to 600° C., according to the degree of tenacity required, allowing them to soak at this temperature for about half an hour and then removing them from the furnace and quenching them in water.

In the case of larger bars, or more complicated shapes, the treatment may be modified somewhat. As a specific example of the treatment of a crank shaft containing about 5 .43% of carbon and about 1.4% of manganese, silicon, sulfur and phosphorus being low, the shaft was heated to a hardening temperature of about 855° C., it was then quenched in water for a period of about one 10 and a quarter minutes, then reheated to about 850° C. and again quenched. The mechanical test obtained from the crank shaft thus treated was as follows:—elastic limit, 34 tons; yield point, 37 tons; breaking load, 15 55 tons; elongation, 24%; reduction of area, 55%; izod test, ft. lbs. 30, angle, 7°.

For an alloy steel of the kind referred to containing say 3% of manganese, the carbon may advantageously be below .5% and it 20 may be down to .2%. Steel thus constituted, after being heat treated as described, and advantageously by heating it to about 800° C., and quenching it in oil and then reheating it to about 650° C. and quenching it in water, 25 yields a material of great commercial value.

Thus, in one example an alloy steel having the following composition: C, .33; Si, .30; Mn, 3.21 when heat treated as just described yielded the following test, namely: 30 elastic limit, 48 tons; yield point, 52 tons; breaking load, 60 tons; elongation, 18%; reduction of area, 40%.

If with about 3% of manganese the carbon be above about .50%, the brittleness of the 35 alloy steel is very marked and the steel would probably not be of much commercial value for purposes such as herein indicated, while if the carbon be below about .2% the resulting material would probably not be of much 40 commercial value for such purposes on account of its greater softness.

Alloy steel of the kind herein described 45 may be produced by refining in an electric furnace, a normally finished carbon steel produced in an open hearth furnace, or by any other suitable process, the desired percentage of manganese being insured by addition, if need be, of manganese in the form, for example, of ferro-manganese at any 50 suitable stage in the manufacture of such steel.

Alloy steels according to the invention, may, in some cases, and for enhancing the 55 qualities thereof for special purposes, include one or more additional metals, for instance nickel, or chromium, or both nickel and chromium, but usually in such cases the proportion of such additional element or elements may be small, say of the order of up to about 1% (one per cent.) of each, or 60 taken together. As such element or elements facilitate the hardening of the alloy steel when the same is heated, and subsequently cooled by quenching, it or they is

or are included in the term hardening metal 65 used in some of the appended claims.

In alloys according to this invention the percentage of carbon may be raised, say for example to about .4 to .6% if the manganese be reduced to below say about 2% and down 70 to about one decimal four per cent.

What I claim is:—

1. An iron manganese alloy steel containing from about decimal two to decimal six 75 of one per cent. of carbon and from about one decimal four to about three decimal five per cent. of manganese.

2. An iron manganese alloy steel containing from about decimal two to decimal six 80 of one per cent. of carbon and from about one decimal four to about three decimal five per cent. of manganese, silicon not exceeding about decimal three of one per cent.

3. An iron manganese alloy steel containing from about decimal two to decimal six 85 of one per cent. of carbon and from about one decimal four to about three decimal five per cent. of manganese, the higher the percentage of manganese the lower being the percentage of carbon, silicon, sulfur and 90 phosphorus being low as set forth.

4. An iron manganese alloy steel containing from about decimal two to decimal three 95 of one per cent. of carbon and from about one decimal four per cent. to about three per cent. of manganese.

5. An iron manganese alloy steel containing from about decimal two to decimal three 100 of one per cent. each of carbon and silicon and from about one decimal four to about two per cent. of manganese.

6. An iron manganese alloy steel containing from about decimal two to decimal six 105 of one per cent. of carbon and about one decimal four per cent. of manganese.

7. An iron manganese alloy steel containing about decimal three of one per cent., each 110 of carbon and silicon and about one decimal four per cent. of manganese.

8. An iron manganese alloy steel containing from about decimal two to decimal six 115 per cent. of carbon from about one decimal four to three decimal five per cent. of manganese and a hardening metal as set forth.

9. An iron manganese alloy steel containing from about decimal two to decimal six 120 per cent. of carbon, from about one decimal four to three decimal five per cent. of manganese and a hardening metal as set forth up to about one per cent.

10. An iron manganese alloy steel capable of offering considerable resistance to tensile and shock stresses, such as is offered by nickel steel chromium steel or nickel chromium steel and containing iron with from 125 about decimal two to decimal six of one per cent. of carbon and from about one decimal four to three decimal five per cent. of man-

- ganese and treated by heat to a relatively high temperature, then rapidly cooled, then reheated to a lower temperature and again cooled.
11. An iron manganese alloy steel capable of offering considerable resistance to tensile and shock stresses such as is offered by nickel steel chromium steel or nickel chromium steel and containing iron with from about decimal two to decimal six of one per cent. of carbon, from about one decimal four to three decimal five per cent. of manganese and a hardening metal up to about one per cent. and treated by heat to a relatively high temperature then rapidly cooled, then reheated to a lower temperature and again cooled.
12. An iron manganese alloy steel capable of offering considerable resistance to tensile and shock stresses, such as is offered by nickel steel, chromium steel or nickel chromium steel and containing iron with from about decimal two to decimal six of one per cent. of carbon and from about one decimal four to three decimal five per cent. of manganese and treated by heat to a temperature of from about 800° to 900° C., then rapidly cooled, then reheated to from about 450° to 700° C. and again cooled.
13. An iron manganese alloy steel capable of offering considerable resistance to tensile and shock stresses such as is offered by nickel steel, chromium steel and nickel chromium steel, containing iron with from about decimal two to decimal five of one per cent.
14. An iron manganese alloy steel capable of offering considerable resistance to tensile and shock stresses such as is offered by nickel steel, chromium steel and nickel chromium steel, containing iron with from about decimal two to decimal five of one per cent. of carbon and from about one decimal four to about two per cent. of manganese and treated by heat to a temperature of from about 800° to 900° C. then rapidly cooled, then reheated to a temperature of from about 450 to 700° C. and then again cooled.
15. As a new article of manufacture, an iron manganese steel alloy low in silicon, sulfur and phosphorus as set forth, containing from about decimal two to decimal six per cent. of carbon and from about one decimal four to three decimal five per cent. of manganese and capable of offering considerable resistance to tensile and shock stresses such as is offered by nickel steel, chromium steel and nickel chromium steel to such stresses.

Signed at London in the county of London, England this twenty ninth day of April 1920.

ROBERT ABBOTT HADFIELD.